

Dec. 11, 1973

TORU KASANAMI ET AL

3,778,389

ELECTRO-CONDUCTIVE MATERIAL CONTAINING PbO AND RuO<sub>2</sub>

Filed Dec. 28, 1970

3 Sheets-Sheet 1



INVENTORS  
TORU KASANAMI  
OSAMU KANO

BY Craig, Antonelli, Stewart & Will

ATTORNEYS

Dec. 11, 1973

TORU KASANAMI ETAL

3,778,389

ELECTRO-CONDUCTIVE MATERIAL CONTAINING PbO AND  $\text{RuO}_2$

Filed Dec. 28, 1970

3 Sheets-Sheet 2



Dec. 11, 1973

TORU KASANAMI ETAL

3,778,389

ELECTRO-CONDUCTIVE MATERIAL CONTAINING PbO AND RuO<sub>2</sub>

Filed Dec. 28, 1970

3 Sheets-Sheet 3



## 1

3,778,389

### ELECTRO-CONDUCTIVE MATERIAL CONTAINING PBO AND RuO<sub>2</sub>

Toru Kasanami and Osamu Kano, Kyoto-fu, Japan, assignors to Murata Manufacturing Co., Ltd., Otokuni-gun, Kyoto-fu, Japan

Filed Dec. 28, 1970, Ser. No. 101,515

Claims priority, application Japan, Dec. 26, 1969,

44/1,062

Int. Cl. H01b 1/06

U.S. Cl. 252—520

25 Claims

### ABSTRACT OF THE DISCLOSURE

An electro-conductive material essentially consisting of a double oxide obtained from PbO and RuO<sub>2</sub> in a molar ratio of 3:1 to 1:3, which is useful as the fundamental composition for production of a resistor paste, a ceramic resistor or the like.

The present invention relates to an electro-conductive material essentially consisting of a double oxide obtained from PbO and RuO<sub>2</sub>, and a resistor composition comprising the same.

Hitherto, there has been known an electro-conductive material essentially consisting of RuO<sub>2</sub>. In a resistor composition obtained by using such known electro-conductive material with a glass frit, the control of the resistivity can be accomplished only by variation of the content of RuO<sub>2</sub>. When the content of RuO<sub>2</sub> is much decreased, however, for production of a resistor composition of high resistance, the content of the crystal component is lessened and a constant dispersibility of the crystal component after sintering is reproduced with great difficulty so that the resistivity of the resistor composition is considerably varied and made uneven on each product. When the content of RuO<sub>2</sub> is much increased for production of a resistor composition of low resistance, the content of the glass component available as a binder is necessarily lowered so that it cannot assure the good rigidity of the resultant resistor composition. The resistor formed with such resistor composition shows an inferior tolerance to moisture in atmosphere, from which the change of the resistivity is caused and the life of the resistor is shortened. Thus, the regulation of the resistivity is not freely made without bringing any disadvantage into the material properties. In addition, a large, positive temperature coefficient of resistivity inherent to RuO<sub>2</sub> appears particularly when the content of RuO<sub>2</sub> is high. Although such an improvement as incorporating Nb<sub>2</sub>O<sub>5</sub> into RuO<sub>2</sub> to make a solid solution was proposed for making flat the temperature characteristics of resistance, it is only effective in making minus the temperature coefficient of resistivity and, for obtaining a low resistance, a large content of RuO<sub>2</sub> than that required in case of RuO<sub>2</sub> alone is necessitated. As stated above, the use of RuO<sub>2</sub> in a too large content is clearly unfavorable, because the rigidity of the resulting resistor is lost.

According to the present invention, which overcomes the above disadvantages, there is used an electro-conductive material essentially consisting of a double oxide ob-

## 2

tained from PbO and RuO<sub>2</sub> in a molar ratio of 3:1 to 1:3 with or without replacing less than 50% by mol of PbO and/or RuO<sub>2</sub> by any other replaceable metal oxide. When the production of high resistance is desired, for instance, less than 50% by mol of RuO<sub>2</sub> may be replaced by Ta<sub>2</sub>O<sub>5</sub> (1/2 Ta<sub>2</sub>O<sub>5</sub>), so that the resistivity of the electro-conductive material itself will be increased. Thus, the content of the electro-conductive material in a resistor composition is not required to make small and, as a matter of course, the defect due to the low content of the electro-conductive material as seen in a conventional resistor composition using the electro-conductive material consisting of RuO<sub>2</sub> alone is overcome.

Further, PbO which is one of the essential components in the electro-conductive material of the invention serves not only as a constituent of the double oxide but also as a binder for the crystal component and the glass component. Because of this reason, a resistor composition produced by the use of the electro-conductive material of the invention is provided with an excellent rigidity even when Nb is incorporated for making minus the temperature coefficient of resistivity.

Furthermore, it may be noted that, compared with RuO<sub>2</sub> alone, the double oxide of PbO and RuO<sub>2</sub> can be dissolved with ease into a glass component at a high temperature and, when cooled, recrystallized to form a crystallized glass material which is thermally and mechanically stable. The thus obtained resistor composition is assured a good contact of the crystal component and of low resistance.

In addition to the above advantages, it may be also noted that the electro-conductive material of the present invention can be utilized for the formation of a ceramic resistor. Compared with a known carbon solid resistor, the ceramic resistor is much more stable to heat and of a higher wattage.

The electro-conductive material of the present invention essentially consists of PbO and RuO<sub>2</sub> in a molar ratio of 3:1 to 1:3, favorably of 1.5:1 to 1:1.5. If necessary, less than 50% by mol of PbO and/or of RuO<sub>2</sub> may be replaced by Bi<sub>2</sub>O<sub>3</sub> (1/2 Bi<sub>2</sub>O<sub>3</sub>) and IrO<sub>2</sub>, respectively. Thus, at least the following four systems may be designed for the electro-conductive material of the invention: (1) PbO-RuO<sub>2</sub>; (2) Bi<sub>2</sub>O<sub>3</sub>-PbO-RuO<sub>2</sub>; (3) PbO-RuO<sub>2</sub>-IrO<sub>2</sub>; (4) Bi<sub>2</sub>O<sub>3</sub>-PbO-RuO<sub>2</sub>-IrO<sub>2</sub>.

For the preparation of the electro-conductive material of the invention, a mixture of the component materials and/or their sources may be sintered, for instance, at a temperature from 400° C. to 1100° C. In the alternative, the electro-conductive material may be produced in a conventional deposition procedure from aqueous solution, if necessary, followed by sintering of the deposited material.

The electro-conductive material of the invention can be used for a wide variety of use. Among them, the use as a resistor paste is one preferred example.

For such use, the electro-conductive material is admixed with a glass frit, an organic binder and a solvent. As the electro-conductive material, there may be used the double oxide of any system as above mentioned, if necessary, with replacement of less than 50% by mol of RuO<sub>2</sub> and/or of PbO by TeO<sub>2</sub>, WO<sub>3</sub>, V<sub>2</sub>O<sub>5</sub>, TiO<sub>2</sub>, MnO<sub>2</sub>, SnO<sub>2</sub>, Sb<sub>2</sub>O<sub>3</sub>, Sb<sub>2</sub>O<sub>5</sub>, CuO, ZnO, Nd<sub>2</sub>O<sub>3</sub>, In<sub>2</sub>O<sub>3</sub>, Nb<sub>2</sub>O<sub>5</sub>,

$Ta_2O_5$  and/or the like. When a resistor paste of high resistance is desired, there may be employed, for instance, the electro-conductive material wherein  $Ta_2O_5$  is incorporated as a replaceable oxide. In case of a resistor paste of low resistance being desired, the electro-conductive material wherein  $Nb_2O_5$  is incorporated as a replaceable oxide may be employed.

Examples of the glass frit are the glass systems of borate, silicate and borosilicate containing at least one of  $Bi_2O_3$ ,  $PbO$ ,  $Al_2O_3$ ,  $ZnO$ ,  $CdO$ , alkali metal oxides, alkaline earth metal oxides and rare earth metal oxides. In order to obtain a resistor paste of high resistance, the use of a frit of  $PbO$ - $B_2O_3$ - $SiO_2$  system glass is recommended. For obtaining a resistor paste of low resistance, the use of a frit of  $Bi_2O_3$ - $PbO$ - $B_2O_3$ - $SiO_2$  system glass is preferred.

As the organic binder, there may be used ethyl cellulose, nitrocellulose or the like. Examples of the solvent include organic solvents such as butyl Carbitol, butyl Carbitol acetate and terpineol.

The molar ratio of the electro-conductive material and the glass frit is usually within a range of 0.5:1 to 0.02:1. In the resistor paste, the combined amount of the organic binder and the solvent normally does not exceed 50% by weight of the total composition.

Another preferred example of the use is a ceramic resistor. Thus, either one of the said systems for the electro-conductive material of the invention is sintered, usually at a temperature from 400° C. to 1300° C. to give a ceramic resistor. If desired, any additive such as  $TeO_2$ ,  $WO_3$ ,  $V_2O_5$ ,  $TiO_2$ ,  $MnO_2$ ,  $SnO_2$ ,  $Sb_2O_3$ ,  $Sb_2O_5$ ,  $CuO$ ,  $ZnO$ ,  $Nd_2O_3$ ,  $In_2O_3$ ,  $Nb_2O_5$ ,  $Ta_2O_5$  or the like may be incorporated prior to the sintering for regulating the resistivity, the resistance temperature characteristics and the sintering temperature. Among them, the use of  $Ta_2O_5$  or  $Nb_2O_5$  is particularly preferred. The amount of the additive to be incorporated may be usually 90% by mol or less on the basis of the combined amount with the electro-conductive material.

Practical and presently preferred embodiments of the present invention are illustratively shown in the following examples.

### EXAMPLE 1

#### Production of electro-conductive material of low resistance

(A)  $PbO$ - $RuO_2$  system.—In a polyvinyl chloride made pot mill with agate balls,  $Pb_3O_4$  and  $RuO_2$  in a molar ratio of 3:1 to 1:3 (in terms of  $PbO$ : $RuO_2$ ) are admixed with water. After evaporation of water, the resultant mixture is admixed in an alumina crucible, heated to 650° C. with a rate of 3° C./min. and calcinated at the temperature for 1 hour to give an electro-conductive material of low resistance as black powder.

When the molar ratio of  $PbO$  to  $RuO_2$  is higher than 1.5, there is remained unreacted  $PbO$  in the resulting product. When the molar ratio of  $RuO_2$  to  $PbO$  is higher than 1.5, excess of  $RuO_2$  remains as unreacted.

(B)  $PbO$ - $RuO_2$ - $Bi_2O_3$  or  $IrO_2$  system.—An electro-conductive material is produced according to the same procedure as in (A) but replacing less than 50% by mol of  $PbO$  by  $Bi_2O_3$  or less than 50% by mol of  $RuO_2$  by  $IrO_2$ . The resulting product is of low resistance.

In the above procedure, the replacement of more than 50% by mol of  $PbO$  by  $Bi_2O_3$  results unfavorably in growth of the particles of the calcinated product. Further, the sintering of the calcinated product affords the grown grains.

### EXAMPLE 2

#### Production of glaze resistor paste

(A)  $PbO$ - $RuO_2$  glaze resistor paste.—The electro-conductive material prepared as in Example 1(A) and a

frit of lead borosilicate glass ( $PbO$  30% by mol;  $B_2O_3$ , 45% by mol;  $SiO_2$ , 25% by mol; molecular weight, 113.30) in a molar ratio of 0.4 to 0.025:1 are admixed with ethyl cellulose in 1.5% by weight and  $\alpha$ -terpineol in 30% by weight on the basis of the combined weight of the electro-conductive material and the glass frit to give a resistor paste.

The resistor paste is printed in a size of 3 mm. x 3 mm. bridging a pair of silver electrodes provided on an alumina ceramics substrate and fired at a peak firing temperature of 680° C. to 880° C. for 10 minutes with a total cycle of 60 minutes. The sheet resistivity with the peak firing temperature and the molar amount of the electro-conductive material is shown in FIG. 1. The sheet resistivity, the cold temperature coefficient of resistivity (-55° C. to +25° C.), the hot temperature coefficient of resistivity (+25° C. to +150° C.) and the voltage coefficient of resistivity with the molar amount of the electro-conductive material to 1 mol of the glass component when fired at 760° C. are shown in Table 1.

TABLE 1

| Molar ratio of electro-conductive material to glass component | Sheet resistivity (Ω/sq.) | T.C.R. (p.p.m./°C.) |      | V.C.R. (percent/V) |
|---------------------------------------------------------------|---------------------------|---------------------|------|--------------------|
|                                                               |                           | Cold                | Hot  |                    |
| 0.4.....                                                      | 633                       | +658                | +612 | +0.0053            |
| 0.3.....                                                      | 2,253                     | +471                | +458 | +0.0021            |
| 0.2.....                                                      | 7,730                     | +186                | +153 | -0.0024            |
| 0.1.....                                                      | 14,780                    | +96                 | +73  | -0.0051            |
| 0.05.....                                                     | 2,347                     | +716                | +645 | -0.0032            |
| 0.025.....                                                    | 1,986                     | +897                | +894 | -0.0012            |

From the above table, it is seen that, in case of the molar ratio of the electro-conductive material being small as around 0.05 or less, the resistivity is lowered and the temperature coefficient of resistivity with positive characteristics is much increased. When the molar ratio is higher than 0.3, the temperature coefficient of resistivity is positive. At the molar ratio of 0.4, the rigidity of the resistor is inferior.

(B) Glaze resistor paste of high resistance.—An electro-conductive material is produced as in Example 1(A) but replacing less than 50% by mol of  $RuO_2$  by  $Ta_2O_5$ . The resulting product becomes grayish with the increase of the  $Ta_2O_5$  content. The employed  $Ta_2O_5$  is served partly to form a solid solution with the  $PbO$ - $RuO_2$  system double oxide and partly to produce a  $PbO$ - $Ta_2O_5$  system double oxide (e.g.  $3PbO$ - $2Ta_2O_5$ ).

The electro-conductive material (0.2 mol) and the glass frit as in (A) (1 mol) are mixed with ethyl cellulose in 1.5% by weight and  $\alpha$ -terpineol in 30% by weight on the basis of the combined weight of the electro-conductive material and the glass frit to produce a glaze resistor paste.

In the similar manner, there are produced electro-conductive materials and glaze resistor pastes using  $TiO_2$  or  $SnO_2$  in place of  $Ta_2O_5$ .

The above obtained glaze resistor pastes are printed and fired as in (A). The sheet resistivity is shown in FIG. 2. The sheet resistivity, the hot temperature coefficient of resistivity, the cold temperature coefficient of resistivity and the voltage coefficient of resistivity with the molar ratio of the electro-conductive material to the glass component when fired at 760° C. are shown in Table 2.

The load life test (70° C. in air; resistor size, 3 mm. x 3 mm. squares; substrate size, 10 mm. x 10 mm.; power, 1/2 w.; 1/2 hrs. ON-1/2 hr. OFF; after 3000 hrs.), the high temperature exposure test (no load: 150° C. in air; after 3000 hrs.), the short time overload test (1 1/4 w. for 5 sec.), the humidity exposure test (40° C.; relative humidity, 95%; after 1000 hrs.) and the noise test (using a resistor noise tester model 315 manufactured by Quan. Tech. Laboratories) are carried out, and the results are shown in Table 3.

TABLE 2

| Electro-conductive material (molar ratio)                                       | Sheet resistivity (K $\Omega$ /sq.) | T.C.R. (p.p.m./ $^{\circ}$ C.) |      | V.C.R. (percent/V.) |
|---------------------------------------------------------------------------------|-------------------------------------|--------------------------------|------|---------------------|
|                                                                                 |                                     | Cold                           | Hot  |                     |
| PbO-RuO <sub>2</sub> (1:1)                                                      | 7.730                               | +156                           | +153 | -0.0024             |
| PbO-RuO <sub>2</sub> - $\frac{1}{2}$ Ta <sub>2</sub> O <sub>5</sub> (1/0.9/0.1) | 69.53                               | -101                           | -36  | -0.0027             |
| PbO-RuO <sub>2</sub> - $\frac{1}{2}$ Ta <sub>2</sub> O <sub>5</sub> (1/0.8/0.2) | 998.2                               | -158                           | -210 | -0.0042             |
| PbO-RuO <sub>2</sub> - $\frac{1}{2}$ Ta <sub>2</sub> O <sub>5</sub> (1/0.7/0.3) | 3,256.0                             | -465                           | -415 | -0.0095             |
| PbO-RuO <sub>2</sub> -TiO <sub>2</sub> (1/0.9/0.1)                              | 157.65                              | -130                           | -115 | -0.0035             |
| PbO-RuO <sub>2</sub> -SnO <sub>2</sub> (1:0.9:0.1)                              | 10.874                              | +165                           | +135 | -0.0022             |

TABLE 3

| Electro-conductive material (molar ratio)                                       | $\Delta R$ (percent) |                           |                     |                   |                   |
|---------------------------------------------------------------------------------|----------------------|---------------------------|---------------------|-------------------|-------------------|
|                                                                                 | Load life            | High temperature exposure | Short time overload | Humidity exposure | Noise (db/decade) |
| PbO-RuO <sub>2</sub> (1:1)                                                      | 0.53                 | 0.23                      | 0.02                | 0.08              | -13.5             |
| PbO-RuO <sub>2</sub> - $\frac{1}{2}$ Ta <sub>2</sub> O <sub>5</sub> (1:0.9:0.1) | 0.26                 | 0.08                      | 0.05                | 0.05              | -3.8              |
| PbO-RuO <sub>2</sub> - $\frac{1}{2}$ Ta <sub>2</sub> O <sub>5</sub> (1:0.8:0.2) | 0.38                 | 0.09                      | 0.07                | 0.23              | +11.5             |
| PbO-RuO <sub>2</sub> - $\frac{1}{2}$ Ta <sub>2</sub> O <sub>5</sub> (1:0.7:0.3) | 0.45                 | 0.19                      | 0.02                | 0.21              | -                 |
| PbO-RuO <sub>2</sub> (1:0.9:0.1)                                                | 0.37                 | 0.27                      | 0.06                | 0.16              | +2.5              |
| PbO-RuO <sub>2</sub> -SnO <sub>2</sub> (1:0.9:0.1)                              | 0.56                 | 0.43                      | 0.08                | 0.98              | -8.3              |

From the above tables, it is understood that the resistors formed as above are excellent in resistance to heat and humidity and quite stable to load.

(C) Glaze resistor paste of low resistance.—An electro-conductive material is produced as in Example 1(A) but replacing less than 50% by mol of RuO<sub>2</sub> by Nb<sub>2</sub>O<sub>5</sub>. The resulting product becomes grayish with the increase of the

x 3 mm. squares; substrate size, 10 mm. x 10 mm.; power,  $\frac{1}{2}$  w.; 1½ hrs. ON=½ hr. OFF; after 3000 hrs.), the high temperature exposure test (no load; 150° C. in air; after 3000 hrs.), the short time overload test (1¼ w. for 5 sec.) and the humidity exposure test (40° C.; relative humidity, 95%; after 1000 hrs.) are carried out, and the results are shown in Table 5.

TABLE 4

| Electro-conductive material (molar ratio)                                                          | Molar ratio <sup>1</sup> | Sheet resistivity (K $\Omega$ /sq.) | T.C.R. (p.p.m./ $^{\circ}$ C.) |      | Noise (db/decade) |
|----------------------------------------------------------------------------------------------------|--------------------------|-------------------------------------|--------------------------------|------|-------------------|
|                                                                                                    |                          |                                     | Cold                           | Hot  |                   |
| PbO-RuO <sub>2</sub> - $\frac{1}{2}$ Nb <sub>2</sub> O <sub>5</sub> (1:0.9:0.1)                    | 0.2                      | 10,832                              | -230                           | -186 | -0.0023           |
| PbO-RuO <sub>2</sub> - $\frac{1}{2}$ Nb <sub>2</sub> O <sub>5</sub> (1:0.95:0.05)                  | 0.3                      | 796.4                               | -15                            | -35  | -0.0016           |
| PbO-RuO <sub>2</sub> - $\frac{1}{2}$ Nb <sub>2</sub> O <sub>5</sub> (1:0.95:0.05)                  | 0.4                      | 74.63                               | +120                           | +178 | -0.0024           |
| PbO-RuO <sub>2</sub> - $\frac{1}{2}$ Nb <sub>2</sub> O <sub>5</sub> (1:0.95:0.05) + Ag, Pd, Au, Pt | 0.4                      | 31.88                               | +321                           | +270 | +0.0035           |

<sup>1</sup> Of electro-conductive material to glass component.

TABLE 5

| Electro-conductive material (molar ratio)                                                             | Load life | $\Delta R$ (percent)      |                     |                   |
|-------------------------------------------------------------------------------------------------------|-----------|---------------------------|---------------------|-------------------|
|                                                                                                       |           | High temperature exposure | Short time overload | Humidity exposure |
| PbO-RuO <sub>2</sub> - $\frac{1}{2}$ Nb <sub>2</sub> O <sub>5</sub> (1:0.9:0.1)                       | 0.37      | 0.14                      | 0.03                | 0.08              |
| PbO-RuO <sub>2</sub> - $\frac{1}{2}$ Nb <sub>2</sub> O <sub>5</sub> (1:0.95:0.05)                     | 0.28      | 0.07                      | 0.02                | 0.07              |
| PbO-RuO <sub>2</sub> - $\frac{1}{2}$ Nb <sub>2</sub> O <sub>5</sub> (1:0.95:0.05)                     | 0.27      | 0.09                      | 0.08                | 0.09              |
| PbO-RuO <sub>2</sub> - $\frac{1}{2}$ Nb <sub>2</sub> O <sub>5</sub> (1:0.95:0.05) plus Ag, Pd, Au, Pt | 0.52      | 0.21                      | 0.13                | 0.35              |

Nb<sub>2</sub>O<sub>5</sub> content. The employed Nb<sub>2</sub>O<sub>5</sub> is served partly to form a solid solution with the PbO-RuO<sub>2</sub> system double oxide and partly to produce a PbO-Nb<sub>2</sub>O<sub>5</sub> system double oxide (e.g. 3PbO-2Nb<sub>2</sub>O<sub>5</sub>).

The electro-conductive material (0.2 mol, and 0.3 mol or 0.4 mol) and a frit of bismuth borosilicate glass (PbO, 20% by mol;  $\frac{1}{2}$ Bi<sub>2</sub>O<sub>3</sub>, 10% by mol; B<sub>2</sub>O<sub>3</sub>, 45% by mol; SiO<sub>2</sub>, 25% by mol) (1 mol) are mixed with ethyl cellulose in 1.5% by weight  $\alpha$ -terpineol in 30% by weight on the basis of the combined weight of the electro-conductive material and the glass frit produces a glaze resistor paste.

Separately, the electro-conductive material (0.4 mol) and the glass frit as above (1 mol) are mixed with 1.5% by weight of ethyl cellulose, 30% by weight of  $\alpha$ -terpineol, 5% by weight of silver powder and 5% by weight of noble metal mixtures (Au:Pd:Pt=10:3:5 by weight) in the form of a dispersion (Au, 10% by weight; Pr, 3% by weight; Pt, 5% by weight; resin, 40% by weight; solvent, 42% by weight) on the basis of the combined weight of the electro-conductive material and the glass frit to produce a glaze resistor paste.

The above obtained glaze resistor pastes are printed and fired as in (A). The sheet resistivity is shown in FIG. 3. The sheet resistivity, the hot temperature coefficient of resistivity, the cold temperature coefficient of resistivity, the voltage coefficient of resistivity and the noise with the molar ratio of the electro-conductive material to the glass component when fired at 760° C. are shown in Table 4.

The load life test (70° C. in air; resistor size, 3 mm.

### EXAMPLE 3

#### Ceramic resistor

(A) Ceramic resistor of low resistance.—The electro-conductive material as prepared in Example 1(A) or 50 1(B) is admixed with polyvinyl methyl ether in 5% by weight on the basis of the weight of the electro-conductive material in the presence of water by a wet procedure and, after evaporation of water, the resulting mixture is molded under a pressure of 700 kg./cm.<sup>2</sup>. The molded product is heated to 900° C. with a rate of 3° C./min. and sintered in air at the temperature for 1 hour. The resistivity of the sintered product is shown in Table 6.

TABLE 6

| Electro-conductive material (molar ratio):                                      | Resistivity (Ω-cm.)  |
|---------------------------------------------------------------------------------|----------------------|
| PbO-RuO <sub>2</sub> (3:1)                                                      | $7.8 \times 10^{-3}$ |
| PbO-RuO <sub>2</sub> (2:1)                                                      | $4.8 \times 10^{-3}$ |
| PbO-RuO <sub>2</sub> (1:1)                                                      | $3.5 \times 10^{-3}$ |
| PbO-RuO <sub>2</sub> (1:2)                                                      | $7.5 \times 10^{-3}$ |
| PbO-RuO <sub>2</sub> (1:3)                                                      | $6.3 \times 10^{-1}$ |
| PbO- $\frac{1}{2}$ Bi <sub>2</sub> O <sub>3</sub> -RuO <sub>2</sub> (0.5:0.5:2) | $6.3 \times 10^{-2}$ |
| PbO- $\frac{1}{2}$ Bi <sub>2</sub> O <sub>3</sub> -RuO <sub>2</sub> (0.5:0.5:1) | $4.6 \times 10^{-3}$ |
| PbO- $\frac{1}{2}$ Bi <sub>2</sub> O <sub>3</sub> -RuO <sub>2</sub> (1:0.5:1.5) | $7.2 \times 10^{-3}$ |
| PbO- $\frac{1}{2}$ Bi <sub>2</sub> O <sub>3</sub> -RuO <sub>2</sub> (2:0.5:1.5) | $8.3 \times 10^{-3}$ |
| PbO-RuO <sub>2</sub> -IrO <sub>2</sub> (1:1:1)                                  | $5.1 \times 10^{-3}$ |
| PbO-RuO <sub>2</sub> -IrO <sub>2</sub> (1:0.5:0.5)                              | $2.3 \times 10^{-3}$ |
| PbO-RuO <sub>2</sub> -IrO <sub>2</sub> (2:1:0.5)                                | $4.3 \times 10^{-3}$ |
| PbO-RuO <sub>2</sub> -IrO <sub>2</sub> (3:1:0.5)                                | $9.8 \times 10^{-3}$ |

(B) Ceramic resistor.—For preparation of ceramic resistors of high resistance, there are used electro-conductive materials of  $\text{PbO}-\text{RuO}_2$  and  $\text{PbO}-\text{RuO}_2-\text{IrO}_2$  systems wherein  $\text{RuO}_2$  or  $\text{IrO}_2$  is partly replaced by  $\text{Ta}_2\text{O}_5$ ,  $\text{Nb}_2\text{O}_5$ ,  $\text{TeO}_2$ ,  $\text{WO}_3$ ,  $\text{V}_2\text{O}_5$ ,  $\text{TiO}_2$ ,  $\text{MnO}_2$ ,  $\text{Sb}_2\text{O}_3$ ,  $\text{SnO}_2$ ,  $\text{ZnO}$ ,  $\text{Nd}_2\text{O}_3$ , or  $\text{In}_2\text{O}_3$ , which are produced from  $\text{Pb}_3\text{O}_4$ ,  $\text{RuO}_2$  and various oxides as shown in Table 7 according to the procedure as in Example 1(A). But,  $\text{Nd}_2\text{O}_3$  is used in the form of  $\text{Nd}_2(\text{CO}_3)_3 \cdot 8\text{H}_2\text{O}$ . The electroconductive material or a mixture of the electro-conductive material (0.8 mol) and the glass frit (0.2 mol) is admixed with polyvinyl methyl ether in 5% by weight on the basis of the weight of the electro-conductive material or the said mixture in the presence of water by a wet procedure, and the resulting mixture is dried, molded and sintered at 900° C. for 1 hour. The thus obtained ceramics is shaped in a size of 2 mm. x 1 mm x 12 mm., a silver paste is applied on both of the opposite sides of the longest direction and fired at 750° C., followed by providing a lead wire to make a ceramic resistor. The temperature coefficient of resistivity and the voltage coefficient of resistivity are shown in Table 7, and the results of the load life test, the high temperature exposure test and the short time overload test are shown in Table 8.

TABLE 7

| Electro-conductive material (molar ratio)                                                                    | Glass frit (mol) | Resistivity (Ω) | T.C.R. (p.p.m./° C.) |        |
|--------------------------------------------------------------------------------------------------------------|------------------|-----------------|----------------------|--------|
|                                                                                                              |                  |                 | Hot                  | Cold   |
| $\text{PbO}-\text{RuO}_2-\frac{1}{2}\text{Ta}_2\text{O}_5(1:0.5:0.5)$                                        | 0.2              | 74.43           | +940                 | +490   |
| $\text{PbO}-\text{RuO}_2-\frac{1}{2}\text{Ta}_2\text{O}_5(1:0.4:0.6)$                                        | 0.2              | 165.4           | +390                 | +270   |
| $\text{PbO}-\text{RuO}_2-\frac{1}{2}\text{Ta}_2\text{O}_5(1:0.3:0.7)$                                        | 0.2              | 356.4           | +95                  | +27    |
| $\text{PbO}-\text{RuO}_2-\frac{1}{2}\text{Ta}_2\text{O}_5(1:0.2:0.8)$                                        | 0.2              | 1,785.5         | -430                 | -325   |
| $\text{PbO}-\text{RuO}_2-\frac{1}{2}\text{Ta}_2\text{O}_5(1.5:0.3:0.7)$                                      | 0.2              | 163.1           | +360                 | +280   |
| $\text{PbO}-\text{RuO}_2-\frac{1}{2}\text{Nb}_2\text{O}_5(1:0.3:0.7)$                                        | 0.2              | 135.2           | -352                 | -270   |
| $\text{PbO}-\text{RuO}_2-\text{SnO}_2(1:0.3:0.7)$                                                            | 0.2              | 366.4           | -210                 | -461   |
| $\text{PbO}-\frac{1}{2}\text{Bi}_2\text{O}_3-\text{RuO}_2-\frac{1}{2}\text{Ta}_2\text{O}_5(0.5:0.5:0.3:0.7)$ | 0.2              | 353.1           | -517                 | -482   |
| $\text{PbO}-\frac{1}{2}\text{Bi}_2\text{O}_3-\text{RuO}_2-\frac{1}{2}\text{Ta}_2\text{O}_5(1:0.5:0.3:0.7)$   | 0.2              | 465.3           | -365                 | -280   |
| $\text{PbO}-\frac{1}{2}\text{Bi}_2\text{O}_3-\text{RuO}_2-\frac{1}{2}\text{Ta}_2\text{O}_5(1:0.3:0.6:0.1)$   | None             | 16.43           | +1,581               | +1,945 |
| $\text{PbO}-\text{RuO}_2-\frac{1}{2}\text{Ta}_2\text{O}_5-\text{WO}_3(1:0.3:0.6:0.1)$                        | None             | 35.42           | +974                 | +651   |
| $\text{PbO}-\text{RuO}_2-\frac{1}{2}\text{Ta}_2\text{O}_5-\frac{1}{2}\text{Sb}_2\text{O}_3(1:0.3:0.6:0.1)$   | None             | 43.52           | +682                 | +783   |
| $\text{PbO}-\text{RuO}_2-\frac{1}{2}\text{Ta}_2\text{O}_5-\text{MnO}_2(1:0.3:0.6:0.1)$                       | None             | 45.36           | +135                 | +238   |
| $\text{PbO}-\text{RuO}_2-\frac{1}{2}\text{Ta}_2\text{O}_5-\text{TeO}_2(1:0.3:0.6:0.1)$                       | None             | 27.31           | +670                 | +573   |
| $\text{PbO}-\text{RuO}_2-\frac{1}{2}\text{Ta}_2\text{O}_5-\text{TiO}_2(1:0.3:0.6:0.1)$                       | None             | 58.36           | +436                 | +670   |
| $\text{PbO}-\text{CuO}-\text{RuO}_2-\text{TiO}_2(0.9:0.1:0.3:0.6)$                                           | 0.2              | 1,538           | -1,510               | -1,315 |
| $\text{PbO}-\frac{1}{2}\text{Nd}_2\text{O}_3-\text{RuO}_2-\text{SnO}_2(0.9:0.1:0.3:0.6)$                     | 0.2              | 425.3           | -615                 | -537   |
| $\text{PbO}-\text{ZnO}-\text{RuO}_2-\frac{1}{2}\text{Ta}_2\text{O}_5(0.9:0.1:0.3:0.6)$                       | 0.2              | 235.4           | +420                 | +365   |
| $\text{PbO}-\frac{1}{2}\text{In}_2\text{O}_3-\text{RuO}_2-\frac{1}{2}\text{Ta}_2\text{O}_5(0.9:0.1:0.3:0.6)$ | 0.2              | 15,473          | -1,315               | -1,265 |

TABLE 8

| Electro-conductive material (molar ratio)                                                                    | Glass frit (mol) | R (percent) |                           |                     |
|--------------------------------------------------------------------------------------------------------------|------------------|-------------|---------------------------|---------------------|
|                                                                                                              |                  | Load life   | High temperature exposure | Short time overload |
| $\text{PbO}-\text{RuO}_2-\frac{1}{2}\text{Ta}_2\text{O}_5(1:0.5:0.5)$                                        | 0.2              | 0.58        | 0.45                      | 0.13                |
| $\text{PbO}-\text{RuO}_2-\frac{1}{2}\text{Ta}_2\text{O}_5(1:0.4:0.6)$                                        | 0.2              | 0.32        | 0.33                      | 0.15                |
| $\text{PbO}-\text{RuO}_2-\frac{1}{2}\text{Ta}_2\text{O}_5(1:0.3:0.7)$                                        | 0.2              | 0.25        | 0.18                      | 0.17                |
| $\text{PbO}-\text{RuO}_2-\frac{1}{2}\text{Ta}_2\text{O}_5(1:0.2:0.8)$                                        | 0.2              | 0.18        | 0.13                      | 0.20                |
| $\text{PbO}-\text{RuO}_2-\frac{1}{2}\text{Ta}_2\text{O}_5(1.5:0.3:0.7)$                                      | 0.2              | 0.35        | 0.27                      | 0.18                |
| $\text{PbO}-\text{RuO}_2-\frac{1}{2}\text{Nb}_2\text{O}_5(1:0.3:0.7)$                                        | 0.2              | 0.23        | 0.35                      | 0.23                |
| $\text{PbO}-\text{RuO}_2-\text{SnO}_2(1:0.3:0.7)$                                                            | 0.2              | 0.95        | 0.62                      | 0.54                |
| $\text{PbO}-\frac{1}{2}\text{Bi}_2\text{O}_3-\text{RuO}_2-\frac{1}{2}\text{Ta}_2\text{O}_5(0.5:0.5:0.3:0.7)$ | 0.2              | 0.83        | 1.23                      | 0.71                |
| $\text{PbO}-\frac{1}{2}\text{Bi}_2\text{O}_3-\text{RuO}_2-\frac{1}{2}\text{Ta}_2\text{O}_5(1:0.5:0.3:0.7)$   | 0.2              | 0.16        | 0.18                      | 0.02                |
| $\text{PbO}-\text{RuO}_2-\frac{1}{2}\text{Ta}_2\text{O}_5-\frac{1}{2}\text{V}_2\text{O}_5(1:0.3:0.6:0.1)$    | None             | 2.37        | 1.25                      | 0.18                |
| $\text{PbO}-\text{RuO}_2-\frac{1}{2}\text{Ta}_2\text{O}_5-\text{WO}_3(1:0.3:0.6:0.1)$                        | None             | 1.63        | 1.13                      | 0.75                |
| $\text{PbO}-\text{RuO}_2-\frac{1}{2}\text{Ta}_2\text{O}_5-\frac{1}{2}\text{Sb}_2\text{O}_3(1:0.3:0.6:0.1)$   | None             | 0.87        | 0.52                      | 0.42                |
| $\text{PbO}-\text{RuO}_2-\frac{1}{2}\text{Ta}_2\text{O}_5-\text{MnO}_2(1:0.3:0.6:0.1)$                       | None             | 0.95        | 0.83                      | 0.23                |
| $\text{PbO}-\text{RuO}_2-\frac{1}{2}\text{Ta}_2\text{O}_5-\text{TeO}_2(1:0.3:0.6:0.1)$                       | None             | 0.72        | 0.53                      | 0.28                |
| $\text{PbO}-\text{RuO}_2-\frac{1}{2}\text{Ta}_2\text{O}_5-\text{TiO}_2(1:0.3:0.6:0.1)$                       | None             | 2.16        | 1.61                      | 0.37                |
| $\text{PbO}-\text{CuO}-\text{RuO}_2-\text{TiO}_2(0.9:0.1:0.3:0.6)$                                           | 0.2              | 1.35        | 1.42                      | 0.65                |
| $\text{PbO}-\frac{1}{2}\text{Nd}_2\text{O}_3-\text{RuO}_2-\text{SnO}_2(0.9:0.1:0.3:0.6)$                     | 0.2              | 0.98        | 1.21                      | 0.72                |
| $\text{PbO}-\text{ZnO}-\text{RuO}_2-\frac{1}{2}\text{Ta}_2\text{O}_5(0.9:0.1:0.3:0.6)$                       | 0.2              | 2.35        | 2.78                      | 1.65                |
| $\text{PbO}-\frac{1}{2}\text{In}_2\text{O}_3-\text{RuO}_2-\frac{1}{2}\text{Ta}_2\text{O}_5(0.9:0.1:0.3:0.6)$ | 0.2              | 4.51        | 3.23                      | 1.78                |

NOTE.—(1) Load life test =  $\frac{1}{2}$  w., 70° C., 1.5 hrs. ON-0.5 hr. OFF, after 3,000 hrs. (2) High temperature exposure test = 150° W., air, after 3,000 hrs. (3) Short time overload test =  $1\frac{1}{4}$  w., 5 sec.

#### What is claimed is:

1. An electro-conductive material essentially consisting of a double oxide obtained from  $\text{PbO}$  and  $\text{RuO}_2$  in a molar ratio of 3:1 to 1:3.
2. The electro-conductive material according to claim 1, wherein less than 50% by mol of  $\text{PbO}$  is replaced by  $\text{Bi}_2\text{O}_3$ .
3. The electro-conductive material according to claim 1, wherein less than 50% by mol of  $\text{RuO}_2$  is replaced by  $\text{IrO}_2$ .
4. The electro-conductive material according to claim 1, wherein less than 50% by mol of  $\text{PbO}$  and of  $\text{RuO}_2$  are respectively replaced by  $\text{Bi}_2\text{O}_3$  and  $\text{IrO}_2$ .
5. A resistor paste which comprises the electro-conductive material according to claim 1, a glass frit, an organic binder and a solvent.
6. The resistor paste according to claim 5, wherein the glass frit is a frit of borate, silicate or borosilicate glass containing at least one of  $\text{Bi}_2\text{O}_3$ ,  $\text{PbO}$ ,  $\text{Al}_2\text{O}_3$ ,  $\text{ZnO}$ ,  $\text{CdO}$ , alkali metal oxides, alkaline earth metal oxides are rare earth metal oxides.
7. The resistor paste according to claim 5, wherein the glass frit is a frit of  $\text{Bi}_2\text{O}_3-\text{PbO}-\text{B}_2\text{O}_3-\text{SiO}_2$  system glass.
8. The resistor paste according to claim 5, wherein the glass frit is a frit of  $\text{PbO}-\text{B}_2\text{O}_3-\text{SiO}_2$  system glass.
9. The resistor paste according to claim 5, wherein less than 50% by mol of  $\text{RuO}_2$  in the electro-conductive material is replaced by at least one of  $\text{TeO}_2$ ,  $\text{WO}_3$ ,  $\text{V}_2\text{O}_5$ ,  $\text{SnO}_2$ ,  $\text{Sb}_2\text{O}_3$ ,  $\text{Nb}_2\text{O}_5$ ,  $\text{CuO}$ ,  $\text{ZnO}$ ,  $\text{Nd}_2\text{O}_3$ ,  $\text{In}_2\text{O}_3$ ,  $\text{Ta}_2\text{O}_5$  and  $\text{Nb}_2\text{O}_5$ .
10. The resistor paste according to claim 5, wherein less than 50% by mol of  $\text{RuO}_2$  in the electro-conductive material is replaced by  $\text{Nb}_2\text{O}_5$ .
11. The resistor paste according to claim 5, wherein less than 50% by mol of  $\text{RuO}_2$  in the electro-conductive material is replaced by  $\text{Ta}_2\text{O}_5$ .
12. The resistor paste according to claim 5, wherein the molar ratio of the electro-conductive material and the glass frit is 0.5:1 to 0.02:1.
13. The resistor paste according to claim 5, wherein at least one of noble metals and their organic compounds is incorporated.

14. The resistor paste according to claim 13, wherein the noble metal is Ag, Pd, Pt, Au, Rh, Ru or Ir.

15. An electro-conductive material according to claim 1, wherein less than 50% by mol of RuO<sub>2</sub> is replaced by Ta<sub>2</sub>O<sub>5</sub>.

16. The resistor paste according to claim 5, wherein less than 50% by mol of PbO in the electro-conductive material is replaced by at least one metal oxide selected from the group consisting of Bi<sub>2</sub>O<sub>3</sub>, TeO<sub>2</sub>, WO<sub>3</sub>, V<sub>2</sub>O<sub>5</sub>, SnO<sub>2</sub>, Sb<sub>2</sub>O<sub>3</sub>, Sb<sub>2</sub>O<sub>5</sub>, CuO, ZnO, Nd<sub>2</sub>O<sub>3</sub>, Ta<sub>2</sub>O<sub>5</sub> and Nb<sub>2</sub>O<sub>5</sub>.

17. The resistor paste according to claim 5, wherein less than 50% by mol of PbO and of RuO<sub>2</sub> are, respectively, replaced by a metal oxide selected from the group consisting of TeO<sub>2</sub>, WO<sub>3</sub>, V<sub>2</sub>O<sub>5</sub>, SnO<sub>2</sub>, Sb<sub>2</sub>O<sub>3</sub>, Sb<sub>2</sub>O<sub>5</sub>, CuO, ZnO, Nd<sub>2</sub>O<sub>3</sub>, In<sub>2</sub>O<sub>3</sub>, Ta<sub>2</sub>O<sub>5</sub> and Nb<sub>2</sub>O<sub>5</sub> wherein the metal oxides respectively replacing said PbO and RuO<sub>2</sub> are the same or different.

18. A ceramic resistor which comprises a ceramic body comprising the electro-conductive material according to claim 1 which has been fired.

19. The ceramic resistor according to claim 18, wherein less than 50% by mol of RuO<sub>2</sub> in the electro-conductive material is replaced by at least one of TeO<sub>2</sub>, WO<sub>3</sub>, V<sub>2</sub>O<sub>5</sub>, TiO<sub>2</sub>, MnO<sub>2</sub>, SnO<sub>2</sub>, Sb<sub>2</sub>O<sub>3</sub>, Sb<sub>2</sub>O<sub>5</sub>, CuO, ZnO, Nd<sub>2</sub>O<sub>3</sub>, In<sub>2</sub>O<sub>3</sub>, Ta<sub>2</sub>O<sub>5</sub> and Nb<sub>2</sub>O<sub>5</sub>.

20. The ceramic resistor according to claim 18, wherein less than 50% by mol of RuO<sub>2</sub> in the electro-conductive material is replaced by Ta<sub>2</sub>O<sub>5</sub>.

21. The ceramic resistor according to claim 18, wherein less than 50% by mol of RuO<sub>2</sub> in the electro-conductive material is replaced by Nb<sub>2</sub>O<sub>5</sub>.

22. The ceramic resistor according to claim 18, wherein less than 50% by mol of RuO<sub>2</sub> and of PbO in the

electro-conductive material are respectively replaced by Nb<sub>2</sub>O<sub>5</sub> and Bi<sub>2</sub>O<sub>3</sub>.

23. The ceramic resistor according to claim 18, wherein less than 50% by mol of RuO<sub>2</sub> and of PbO in the electro-conductive material are respectively replaced by Ta<sub>2</sub>O<sub>5</sub> and Bi<sub>2</sub>O<sub>3</sub>.

24. The ceramic resistor according to claim 18, wherein less than 50% by mol of PbO in the electro-conductive material is replaced by at least one of Bi<sub>2</sub>O<sub>3</sub>, TeO<sub>2</sub>, WO<sub>3</sub>, V<sub>2</sub>O<sub>5</sub>, SnO<sub>2</sub>, Sb<sub>2</sub>O<sub>3</sub>, Sb<sub>2</sub>O<sub>5</sub>, CuO, ZnO, Nd<sub>2</sub>O<sub>3</sub>, Ta<sub>2</sub>O<sub>5</sub> and Nb<sub>2</sub>O<sub>5</sub>.

25. The ceramic resistor according to claim 18, wherein less than 50% by mol of PbO and of RuO<sub>2</sub> are, respectively, replaced by TeO<sub>2</sub>, WO<sub>3</sub>, V<sub>2</sub>O<sub>5</sub>, SnO<sub>2</sub>, Sb<sub>2</sub>O<sub>3</sub>, Sb<sub>2</sub>O<sub>5</sub>, CuO, ZnO, Nd<sub>2</sub>O<sub>3</sub>, In<sub>2</sub>O<sub>3</sub>, Ta<sub>2</sub>O<sub>5</sub> and Nb<sub>2</sub>O<sub>5</sub> wherein the metal oxides respectively replacing said PbO and RuO<sub>2</sub> are the same or different.

#### References Cited

##### UNITED STATES PATENTS

|           |         |                   |       |         |
|-----------|---------|-------------------|-------|---------|
| 3,373,119 | 3/1968  | Krystyniak        | ----- | 252—518 |
| 3,352,797 | 11/1967 | Kim               | ----- | 252—518 |
| 3,304,199 | 2/1967  | Faber, Sr. et al. | ----- | 252—518 |
| 3,324,049 | 6/1967  | Holmes            | ----- | 252—518 |
| 3,044,901 | 7/1962  | Garnsworthy       | ----- | 252—518 |
| 2,950,996 | 8/1960  | Place, Sr. et al. | ----- | 252—518 |
| 3,052,573 | 9/1962  | Dumesnil          | ----- | 252—518 |

GEORGE F. LESMES, Primary Examiner

J. P. BRAMMER, Assistant Examiner

U.S. Cl. X.R.

117—201; 252—518